

Aug. 7, 1951

**J. CADGENE**  
PROCESS FOR IMPROVING THE CHARACTERISTICS  
OF THERMOPLASTIC FABRICS  
Filed June 17, 1949

2,563,394



FIG. 1.



FIG. 2.

JACQUES CAOGENE  
BY  
Inventor  
Michael S. Bier  
-  
1901

Patented Aug. 7, 1951

卷之三

**2,563,394**

UNITED STATES PATENT OFFICE

**2,563,394**

## PROCESS FOR IMPROVING THE CHARACTERISTICS OF THERMOPLASTIC FABRICS

**Jacques Cadgene, Paterson, N. J.**

Application June 17, 1949, Serial No. 99,786

**1. Claim. (Cl. 8—130.1)**

1

My present invention relates to methods of improving the characteristics of thermoplastic fabrics, more particularly the characteristics of fabrics made of such substances as nylon, vinyl resins, and cellulose acetates.

It is an object of my present invention to improve the dimensional stability of fabrics of the above type.

It is a further object of my present invention to improve the resistance against stretching, creasing and shrinking of fabrics made of thermoplastic substances, particularly consisting of thermoplastic substances of the type specified above.

A further and important object of my present invention consists in finishing treatments for fabrics made of thermoplastic substances which have the characteristic tendency to return, when wetted, into their original shape, said finishing treatment having the purpose of eliminating such tendency so that the treated fabrics permanently retain the shape they assume during such finishing treatment.

With the above objects in view, my present invention mainly consists in methods of improving the characteristics of thermoplastic fabrics of the above defined type which methods include the step of passing the thermoplastic fabric to be treated through a heated bath of a liquid substance which does not adhere to the fabric passed through the bath.

I have found it particularly advantageous to use for the purposes of my present invention a heated molten metal bath and to heat this bath to a temperature sufficient to slightly plasticize the fabrics passed therethrough, but insufficient to melt the same.

Particularly good results are attained with my new processes if the fabrics are subjected to tension during treatment in the metal bath.

In the case of fabrics, the tension is exerted preferably in transversal and longitudinal direction of the longitudinal piece of fabric subjected to treatment.

In general, the time of treatment depends upon the type of plastic material of which the fabrics consist and on the thickness of its yarns. Of course, the temperature of the metal bath has also to be taken into consideration when determining the length of time of immersion of the fabrics into the bath.

Nevertheless, it might be stated that in general the time of treatment, i. e. immersion into the metal bath, varies between three and sixty seconds, depending upon the above listed various conditions influencing the treatment.

2

It has been found that the surface of a molten metal bath has the tendency to oxidize and cause formation of a metal oxide layer on the surface of the molten metal. In order to avoid such oxide layer which adversely affects the treated fabrics it is advisable to provide a zone of inert gas, at least at those surface portions of the metal bath where the fabrics enter and leave the bath, so as to prevent adherence of oxides to the surface of the treated fabrics. Reducing gases, such as carbon monoxide, are particularly well adapted for the purposes of my present invention.

10 the purposes of my present invention.  
The novel features which I consider as characteristic for my invention are set forth in particular in the appended claim. The invention itself, however, both as to its construction and its method of operation, together with additional objects and advantages thereof, will be best understood from the following description of specific 15 embodiments when read in connection with the accompanying drawings, in which:

Fig. 1 is a schematic cross section through a metal bath arrangement adapted for the purposes of my present invention; and

25 Fig. 2 is a schematic showing of a modified metal bath arrangement similar to the one shown in Fig. 1, but equipped with embossing rollers.

The arrangement shown in Figure 1 consists of a vessel 10 made of a heat insulating material in which the electric heating coils 11 are embedded.

This vessel 10 is partly filled with a molten metal alloy 12, heated by means of the heating coils 11.

The vessel is closed on its top by a cover 13 provided with two slots 14 and 15. The fabric 16 to be treated enters the vessel through slot 14, passes over the first metallic supporting roller 17, engaging face 18 of the fabric, and over the second metallic supporting roller 19, engaging the face 20 of the fabric. Then the fabric 16 passes over the guiding roller 21 and is pulled out of the metal bath through the outlet slot 15 by means of the take-up roller 22 exerting tension on the fabric in direction of arrow 23.

45 It should be noted that it is of great importance that the metal rollers 17 and 19 engage both faces 18 and 20, respectively, of the fabric 16, as otherwise the metal particles of the metal bath 12 are unable to properly penetrate and affect all filaments 50 of the fabric. This seems to be due to the fact that air particles are caught between the filaments preventing access of the molten metal to the surface of all filaments and that these air particles are removed by passage of the fabric 55 over the rollers 17 and 19.

The space 24 within the vessel 10 above the surface 25 of the metal bath 12 is preferably filled with a reducing gas, e. g. by introducing through conduit 26 carbon monoxide, preventing formation of an oxide film on the surface 25 of the bath. In order to control the presence of monoxide in the treating vessel, I have found it advisable to provide in the surface of the vessel a small exit opening 27 provided with a valve 28. The monoxide escaping through this opening is lighted and burns with a small flame 29. As long as this flame 29 is visible, there is carbon monoxide in the treating vessel and no danger of formation of an oxide film exists.

The arrangement shown in Figure 2 is very similar to the arrangement shown in Figure 1. The only difference is that the first treating roller 30 in this arrangement is provided with teeth 31 so as to exert a transversal tension upon the fabric to be treated, and the second treating roller 32 has an embossed surface cooperating with the corresponding embossed surface on the roller 33 so as to emboss the fabric during its passage through the metal bath.

It is evident that at the time the fabric passes between the rollers 32 and 33, it is in a slightly plasticized state and easily embossed.

My new processes are carried out in the following way:

First, the vessel 10 is filled with a metal or metal alloy having a low melting point. Eutectic metal alloys are particularly adapted for my purposes. Thus, I have found that alloys composed of cadmium, antimony and lead furnish a very good bath. Similarly, lead, tin, cadmium and similar alloys, such as bismuth, tin, lead alloys, are very well adapted as metal bath compositions.

Then, the vessel 10 is heated by means of the heating coils 11 until the desired metal bath is formed.

Thereafter, a reducing gas, such as carbon monoxide, is introduced through conduit 26, valve 28 is opened, and flame 29 is lighted.

The apparatus is then ready for operation and the fabric is passed through it so that it is immersed into the bath for a time period of between three and sixty seconds.

Several examples of my new process are described below without, however, limiting the scope of my present invention to the particular compositions and conditions set forth in the same:

#### Example I

A nylon fabric is passed under tension through a metal bath consisting of 60% of lead, 20% of tin, and 15% of cadmium. The temperature of this metal bath is maintained at between 115° and 130° C. The speed of movement of the fabric is regulated so that it immerses into the bath for between ten to twelve seconds.

#### Example II

A fabric consisting of cellulose acetate yarn is passed through a bath of the type described in Example I, and moved during its passage between two embossing rollers of the type shown in Figure 2. The entire time of passage amounts to about thirty-five seconds, and the bath is kept at

5 a temperature of about 140° C. The obtained fabric is embossed and, furthermore, made crease and shrinkage resistant.

#### Example III

A fabric of the type defined in Example I is treated as defined in Example II, the only difference being that the two embossing rollers have smooth surfaces. This treatment will result in adhesion of the slightly plasticized yarns of the fabric, permanently connecting them at their points of intersection to each other.

It will be understood that each of the elements described above, or two or more together, may also find a useful application in other types of processes for treating thermoplastic fabrics made thereof, differing from the types described above.

While I have illustrated and described the invention as embodied in processes for finishing nylon and similar fabrics, I do not intend to be limited to the details shown, since various modifications and structural changes may be made without departing in any way from the spirit of my invention.

Without further analysis, the foregoing will so fully reveal the gist of my invention that others can by applying current knowledge readily adapt it for various applications without omitting features that, from the standpoint of prior art, fairly constitute essential characteristics of the generic or specific aspects of this invention, and, therefore, such adaptations should and are intended to be comprehended within the meaning and range of equivalence of the following claim.

What I claim as new and desire to secure by Letters Patent is:

Process of improving the characteristics of knitted and woven fabrics made of thermoplastic yarn consisting of thermoplastic substances such as nylon, vinyl resin, cellulose acetates and like thermoplastic substances, said process comprising the steps of passing an elongated piece of said fabric through a heated molten metal bath having a temperature sufficient to plasticize said fabric, forcing said molten metal of said bath transversely through said fabric by pressing one face of said fabric against one of a pair of spaced rollers and the other face of said fabric against the other of said pair of spaced rollers, while the fabric is immersed in said bath so as to thereby insure contact of said molten metal of said bath with the entire surface of the yarns of which said fabric consists, and subjecting said fabric to both longitudinal and transverse tension while it is immersed in said molten metal bath.

JACQUES CADGENE.

#### REFERENCES CITED

The following references are of record in the file of this patent:

#### UNITED STATES PATENTS

| Number    | Name           | Date          |
|-----------|----------------|---------------|
| 2,334,233 | Wood           | Nov. 15, 1943 |
| 2,346,208 | Conaway        | Apr. 11, 1944 |
| 2,437,687 | Dreyfus et al. | Mar. 16, 1948 |
| 2,437,703 | Moncrieff      | Mar. 16, 1948 |